

## UNITED STATES PATENT OFFICE

ALBERT A. FREY, OF FOREST HILLS, PENNSYLVANIA, AND GUERNSEY H. COLE, OF MIDDLETON, OHIO, ASSIGNEES TO WESTINGHOUSE ELECTRIC AND MANUFACTURING COMPANY, A CORPORATION OF PENNSYLVANIA

## MAGNETIC ALLOY

No Drawing.

Application filed July 17, 1931. Serial No. 551,548.

Our invention relates to alloys and more particularly to magnetic alloys containing iron, silicon and arsenic.

The principal object of our invention is to provide ductile alloy containing iron, silicon and arsenic which, when tested magnetically, has a low core loss.

Another object of our invention is to provide an alloy containing iron, silicon and arsenic that shall have higher ductility than iron-silicon alloys and which, when utilized in cores for transformers, is characterized by having a total watt loss as low as .92 watts per kilogram, when tested at an induction of 10,000 gausses and at 60 cycles.

A further object of our invention is to provide cores for electrical apparatus, such as transformers, generators and the like, comprising rolled and annealed laminations comprising an alloy of iron, silicon and arsenic.

Iron-silicon alloys have heretofore been extensively utilized in the cores of electrical apparatus, such as transformers. When more than 4 per cent silicon, however, is utilized, the alloy becomes brittle and is difficult to roll and punch. Consequently, the amount of silicon which may be utilized is limited. It is essential, in producing magnetic materials, that the material utilized shall have a high electrical resistance in order to reduce eddy-current losses. Silicon is very effective in this respect but, since the amount of this element which may be utilized is small, it is impossible to reduce the eddy current loss beyond a certain limit and still provide an alloy which is workable.

We have made the discovery that the electrical properties of iron-silicon alloys may be considerably improved by the addition of .1 per cent to 6 per cent of arsenic, whereby an alloy is produced which may be rolled and punched. When properly annealed, our improved alloy has a higher maximum permeability than iron-silicon alloys and is characterized by having an especially low core loss.

In practicing our invention, we melt iron in a suitable furnace, such as an electric induction furnace, which is maintained at a temperature of from 2700° F. to 2900° F.

At this temperature, arsenic may be added to the molten iron, either as metallic arsenic or as ferro-arsenic, or it may be introduced by passing a stream of arsenic vapor, arsene or arsenic hydride into the molten iron. After the arsenic has been dissolved in the molten iron, silicon is added, either as pure silicon or ferrosilicon. We prefer, however, to add the arsenic and silicon to the molten iron in one operation, as the iron is being poured into the ladle by the addition of an alloy or compound of arsenic, silicon and iron. The alloy may then be cast into ingots of any desired form to be subsequently rolled into bars or sheets, according to the usual practice.

The amount of arsenic and silicon which are added to the iron will depend upon the magnetic and mechanical characteristics desired and, as a rule, will vary between .1 per cent to 6 per cent of arsenic.

The amount of arsenic utilized will depend upon the magnetic characteristics desired. If a high saturation value is required, a small amount, say not more than  $\frac{1}{2}$  per cent, is sufficient. Arsenic increases the resistance of the alloy without increasing the brittleness and, consequently, when a comparatively large amount of arsenic is utilized, the core loss is decreased.

Arsenic, however, is very difficult to introduce into the alloy because of its high volatility at the alloying temperature of the iron. We, therefore, prefer to utilize an alloy containing from 1 per cent to 2 per cent, by weight, of arsenic. The amount of silicon which may be added is limited because large amounts increase the brittleness of the alloy and render it unforgeable. The amount of silicon, therefore, should be maintained within the range of 3 per cent to 4 per cent, by weight. An alloy containing the arsenic and silicon, within the amounts specified, possesses high fluidity in the molten state and may be readily cast.

After the alloy is cast and rolled, in the manner specified, it is subjected to a suitable annealing operation. A suitable annealing operation may consist in heating the rolled sheets to a temperature of 900° to 1100° C. in air, a neutral atmosphere or in hydrogen.

for a period of from 2 to 8 hours and then cooling in the furnace.

In preparing laminations for electrical apparatus, such as transformers, however, we prefer to anneal the sheet material in air, a neutral atmosphere or hydrogen for a period of several days at a temperature of 900° or 1100° C. The material is cooled in the furnace, the laminations are punched and the material is then re-annealed for a similar period at a temperature of 700° to 800° C.

Our preferred alloy, when properly annealed, has exceptionally good magnetic characteristics. For example, an alloy containing from 1 per cent to 2 per cent, by weight, of arsenic and from 3.5 per cent to 4 per cent, by weight, of silicon, in the form of a rolled sheet, had a core loss of only .92 watts per kilogram when tested at an induction of 10,000 gausses and 60 cycles.

The following table shows the actual analysis and core losses for alloys of different compositions after they have been rolled into sheet form and annealed.

|    | Silicon | Arsenic | Iron  | W <sub>10</sub> (Watt loss per kg. at 60 cycles at an induction of 10,000 gausses) | W <sub>14</sub> (Watt loss per kg. at 60 cycles at an induction of 14,000 gausses) |
|----|---------|---------|-------|------------------------------------------------------------------------------------|------------------------------------------------------------------------------------|
| 25 | %       | %       | %     |                                                                                    |                                                                                    |
| 30 | 4.0     | .75     | 95.25 | 1.03                                                                               | 2.31                                                                               |
|    | 3.72    | .30     | 95.98 | 1.02                                                                               | 2.31                                                                               |
|    | 3.61    | .59     | 95.8  | .96                                                                                | 2.05                                                                               |
|    | 3.48    | .79     | 95.73 | .97                                                                                | 2.17                                                                               |
| 35 | 3.92    | 1.04    | 95.04 | .92                                                                                | 2.01                                                                               |

Our improved magnetic alloys are superior to iron-silicon alloys because a higher content of combined arsenic and silicon may be utilized than of silicon alone, without increasing the brittleness of the alloy. A ductile alloy having a higher resistance than iron-silicon alloys may thus be formed. This is highly essential because it decreases the core loss. The arsenic also acts as a purifier of the alloy, while it is in the molten state, because it reacts with the non-metallic inclusions forming a compound which floats to the surface of the molten alloy and may be removed. Our improved alloy is superior to iron-arsenic alloys because sheets formed from such alloys have the tendency to adhere to each other and to the rolls when a plurality of them are rolled according to the hot-pack rolling process.

While we have disclosed our invention in considerable detail and have given specific examples, it will be understood that the examples are to be construed as illustrative and not by way of limitation. For example, it will be understood that the alloy will contain a small amount of impurities. It is preferred that the amount of magnetically detrimental impurities shall be less than .02 per cent. Electrolytic iron or a high grade com-

mercial iron, such as "Armco" iron, may be utilized. Other elements or impurities may be present, provided they are not magnetically detrimental.

Other modifications will become apparent to those skilled in the art without departing from the spirit and scope of our invention. It is, therefore, desired that only such limitations shall be imposed as are indicated in the appended claims.

We claim as our invention:

1. A magnetic alloy comprising iron as a major constituent and silicon and arsenic as minor constituents.

2. A magnetic alloy comprising iron as a major constituent and from 1 per cent to 6 per cent, by weight, of silicon and from .1 per cent to 6 per cent, by weight, of arsenic.

3. A magnetic alloy comprising iron as a major constituent and from 1 per cent to 6 per cent, by weight, of a silicon compound or alloy and from .1 per cent to 6 per cent, by weight, of an arsenic compound or alloy.

4. A magnetic alloy comprising iron as a major constituent and a combined arsenic and silicon content of from .2 per cent to 12 per cent.

5. A magnetic alloy comprising iron as a major constituent and from 3 per cent to 4 per cent, by weight, of silicon and from .5 per cent to 2 per cent, by weight, of arsenic.

6. A magnetic ductile alloy comprising iron as a major constituent and from 1 per cent to 2 per cent, by weight, of arsenic and from 3.5 per cent to 4 per cent, by weight, of silicon, said alloy having a core loss of less than one watt per kilogram at an induction of 10,000 gausses.

7. A magnetic alloy comprising at least 90 per cent, by weight, of iron, from .5 per cent to 2 per cent, by weight, of arsenic and from 1 per cent to 4 per cent, by weight, of silicon, said alloy having a core loss of less than one watt per kilogram when tested at an induction of 10,000 gausses and 60 cycles.

8. An article of manufacture comprising a rolled sheet of magnetic material composed of an alloy comprising at least 90% iron, .1% to 6% silicon and .1% to 6% arsenic.

9. A lamination for electrical apparatus comprising a rolled sheet of magnetic material composed of an alloy comprising at least 90% iron, .1% to 6% silicon and .1% to 6% arsenic.

10. A transformer core composed of a plurality of laminations of magnetic sheet material, each of said sheets being formed of an alloy comprising at least 90% iron, .1% to 6% silicon and .1% to 6% arsenic.

In testimony whereof, we have hereunto subscribed our names.

ALBERT A. FREY.  
GUERNÉY H. COLE.